# EUROPEAN PATENT SPECIFICATION

(11) **EP 0 044 601 B1**
(45) Date of publication and mention of the grant of the patent: **28.05.1986**
(21) Application number: 81200822.5
(22) Date of filing: 20.07.1981
(51) Int. Cl.: D06P 5/15, D06P 1/649

(54) **Process for discharge printing of polyester materials**
Verfahren zum Ätzen von Polyestermaterialen
Procédé d'impression par rongeage de matières polyesters

(30) Priority: 18.07.1980 NL 8004160
(43) Date of publication of application: 27.01.1982
(73) Proprietor: EPEC-DINON, NL-7545 GW Enschede (NL)
(72) Inventor: Spierdijk, Ronald Johannes, NL-7545 GW Enschede (NL); Veltman, Willem Laurens, NL-3062 TL Rotterdam (NL); Weerkamp, Louis Leonard, NL-7544 KV Enschede (NL)
(74) Representative: van der Veken, Johannes Adriaan

## Description

The invention relates to a process for printing polyester containing textile materials by applying in one step wet on wet a first composition containing at least a dischargeable dye and a discharge composition containing a compound discharging said dischargeable dye onto a fabric, drying the fabric and fixing the dyes by heating.

Such a process for printing polyester or polyester/cotton fabrics in one step using a first composition containing a dischargeable dye and urea (thiourea is used for other fabrics) and a discharging composition containing only high amounts of stannous chloride and sodium sulphoxylate formaldehyde as discharging agent is known from GB-A-1.508.855.

However, the use of a high concentration of the discharging agent such as stannous chloride or zinc sulphoxylate formaldehyde presents the disadvantage that
a) a small dying range is obtained as if more stannous chloride or sulphoxylate is used, the less dyes are dischargeproof. In practice, this results in printed fabrics having dischargeproof dyes which are relatively dull in colour.
b) When the dyes are fixed on the textile material hydrochloric acid escapes from stannous chloride during this reaction mechanism which gives rise to high corrosion and attack of the metal of the steamer in which the fixation takes place.
c) Stannous chloride and zinc sulphoxylate formaldehyde are expensive products so that the process is very costly.

It is now the aim of the invention to provide a process for printing of polyester containing textile materials by applying a discharging agent whereby the abovementioned disadvantages do not arise and, in particular, improved colour patterns can be obtained with an appreciable saving in raw materials. The opportunity is also created for discharging textile materials without using any stannous chloride, depending on the dyes and materials to be processed.

This aim is attained in that the dischargeable dye is discharged by a thiourea or isothiourea compound present in the discharge composition.

In this way the following advantages are obtained:
a) A more extensive range of dyes can be used as more dyes will be proof to the discharging agent in the form of an thiourea or an isothiourea compound.
b) Owing to the fact that no or at least less stannous chloride need be used, less corrosion of the installation takes place.
c) Through an appreciable smaller use of stann ous chloride or even without stannous chloride important economic advantages are obtained.
d) A multi-colured design can be obtained by making use of masks both in the stencils for the first composition and the stencils for applying the discharging composition, which may contain a second colour being proof against the discharging compound thiourea or isothiourea.
e) The textile material need be passed over a printing machine once only, while drying after applying the first dye-containing composition can be omitted; this leads to major economic advantages.
f) Since the drying of the first colour-containing composition is superfluous, no additional problems can result with parts of the textile material containing dye already fixed, so that the percentage of waste is reduced.
g) The composition containing the first dye and the discharging composition can be printed in relation to each other so that the opportunities for design and artistic work are much greater. In particular, this process allows designs hitherto impossible to be printed onto textile materials.
h) Single-stage printing allows thicker, coarser polyester qualities to be worked with.

It should be noted that GB-A-1.440.904 discloses a printing process wherein a composition containing at least one dischargeable dye is applied onto fabric of polyester fibres and after dying the polyester material a discharging composition is applied containing 7 parts by weight of stannous chloride and 5 parts by weight of an amine binding hydrochloric acid evolved in the action of stannous chloride. This amine may be urea or thiourea. Subsequently the fabric is subjected to a steam treatment with superheated steam at a temperature of 180°C for 10 minutes for fixing the dyes. This process does not provide multicoloured designs of good quality.

DE-B-1.103.288 also describes a discharge printing process for printing cellulose ester containing fabrics by applying a two steps process, the discharging composition containing 15 parts by weight of sodium sulphoxylate formaldehyde as discharging agent and 10 parts by weight of thiourea. This process does not provide multicoloured design of good quality.

US-A-2.874.022 discloses the use of a discharging composition containing sodium sulphoxylate formaldehyde and thiourea for discharge printing cellulose acetate in two steps.

Chemical Abstracts, Vol. 93, no. 12, September 1980, page 63 no. 115853t describes discharge printing of acrylic fibres in two steps using a discharge composition containing stannous chloride as a dye discharging agent and thiourea.

DE-A-2.727.327 and CH-A-612.307 describes a two step discharge printing process for polyester fabric the discharge composition containing 8 to 10% of zinc sulphoxylate formaldehyde and 1 to 3% of thiourea.

US-A-3.958.287 describes the use of thiourea as a hydrotroping or neutralizing agent in discharging compositions containing stannous chloride as discharging agent, the printing process is a two step process.

This two-stage method presents the disadvantage, of a high percentage of waste being a consequence of the fact that the process is difficult to check. Moreover, when the dischargeable dye has been applied by means of the first composition and has dried the dischargeable dye may be fixed to the fibres in certain parts of the fabic in such a way that the discharge agent stannous chloride is not able to discharge these parts printed by the first dye. Furthermore, the opportunities for design and artistic work are restricted since the print with the composition containing the discharging agent and the first composition cannot be printed to match in relation to each other, while finally, this process can virtually be applied only on thin polyester-materials.

The discharging composition as used in the invention may contain an additional discharging agent preferably in the form of a salt of a metal of the second to fourth groups of the periodic system. However, this is unnecessary if suitable recipes are applied.

The composition may contain as such an additional discharging agent a halogen compound of a bivalent metal, in particular zinc chloride, and yet more advantageously a halogen compound of a quadrivalent metal, in particular tin, which tin compound is applied in the form of stannous chloride. It is recommended to use at most 5% of such an additional discharging agent.

The discharge composition may contain at most 4% of a dye discharging metal salt preferably of a halide or a halide of a metal of the second to fourth groups of the periodic system as additional discharge agent besides 0,1 to 10%, preferably 0,1 to 5% of a thiourea or isothiourea compound as discharge agent. The metal halide is advantageously zinc or stannous chloride.

A composition may effectively be used for printing which contains 0,1 to 4% of a metal salt, more particularly 0,1 to 2% and 0,5 to 10% of organic discharging agent, still more particularly 1 to 4% and more effectively 0,5 to 1% of a metal salt, preferably stannous II chloride and 0,5 to 5% thiourea.

Preferably after having applied the first and the discharge composition, the fabric is subjected to heat treatment at a temperature exceeding 80°C and less than the decomposing temperature of the textile material, preferably to a steam treatment at a temperature of 150 to 180°C.

The process according to the invention is particularly used for rotation film-printing of textile materials containing synthetic and natural fibres, particularly cellulose fibres (cotton) mixed with polyester.

Preferably a discharge composition for use in the process of the invention contains at most 4% of a dye discharging metal salt preferably of a halide of a halide of a metal of the second to fourth groups of the periodic system as additional discharge agent besides 0,1 to 10%, preferably 0,1 to 5% of a thiourea or isothiourea compound as discharge agent.

The thickeners applied in the composition according to the invention may effectively consist of cellulose or starch derivatives thickening with water. Other solvents can also be included in the composition such as e.g, benzene, in which case semi-emulsions are obtained.

The invention will now be explained by mean of some examples.

### Example I

### Printing of Textile

A layer of one of the discharge-resistant printing pastes as described in one of the Examples II to VI is applied to the textile material to be printed (50% cotton fibre and 50% polyester fibre) and a print overlayer is applied to this of a known printing paste with dischargeable dyes.

Both printing pastes are printed wet on wet in a single stage with the aid of a printing machine.

The cloth is then dried, fixed at e.g. a temperature of 170°C within a period of e.g. 10 minutes, after which the textile material is further treated.

It is recommended that the printing paste according to the invention be first applied to the textile material and then the paste with dischargeable dye, as this produces optimum results.

### Example II

### Discharging Composition for e.g. Dispersed Dyes

360 g of thickener (12% solution) is mixed with 40 g of emulsifier (12,5% solution), 16 g of sodium acetate and 2 g-of citric acid and 48 g of thiourea.

Further, 10 g of carrier and 320 ml of Terpentoi^{O} are added to this composition, together with a desired quantity of discharge-proof dispersed dyes and 20 to 40 g of stannous II chloride (depending on the properties and concentrations present of the dischargeable dyes or those to be discharged). This is filled up to 1000 g with water or another solvent.

### Example III

### Discharging Composition Suitable for e.g. Dispersed Dyes

The composition described in Example II is prepared but without 20-40 g stannous II chloride. Instead of stannous II chloride 30 g of "Solutionsalz"^{@} or an identical product and 30 g of Lyogene V^{@} or an identical product is added. It is filled up to 1000 g with water.

### Example IV

### Discharging Composition Suitable for Dispersed Reactive Dyes

The composition described in Examples II or III is taken but the quantity of citric acid is increased to 50 g and 80 g of polyethyleneglycol (specific weight 300) is also added, after which discharging on to polyester/cotton is possible.

### Example V

### Discharging Composition Suitable for Pigment Dyes

700 g of an acid pigment cover printing paste is taken, to which is added 20 g of sodium acetate, 20 g of fixation agent, 50 g of tylose MH 300 (7% solution), 50 g of citric acid and 50 g of thiourea. A certain quantity of discharge-resistant pigment dye and 20-40 g of stannous II chloride (depending on the properties and dye concentrations present of dischargeable dyes or dyes to be discharged) is further added to this composition. It is filled up to 1000 g with water. By means of this printing paste cover printing is possible on polyester/cotton with discharge-resistant pigment-dyes.

### Example VI

### Discharge Composition Suitable for Pigment Dyes

The composition described in Example V is taken but without 20-40 g of stannous II chloride and, instead, the products named in Example III are added.

## Claims

1. A process for printing polyester containing textile materials by applying in one step wet on wet a first composition containing at least a dischargeable dye and a discharge composition containing a compound discharging said dischargeable dye onto a fabric drying the fabric and fixing the dyes by heating, characterized in that the dischargeable dye is discharged by a thiourea or isothiourea compound present in the discharge composition.

2. A process according to claim 1, characterized in that the discharge composition contains at most 4% of a dye discharging metal salt as additional discharge agent besides 0,1 to 10%, of thiourea or isothiourea compound as discharge agent.

3. A process according to claim 2, characterized in that the dye discharging metal salt is a halide of a metal of the second to fourth group of the Periodic System.

4. A process according to claim 2 or 3, characterized in that the discharge composition contains 0,1 to 5% of a thiourea or isothiourea compound as discharge agent.

5. A process according to claim 2-4, characterized in that the metal halide is zinc or stannous chloride.

6. A process according to any one of the preceding claims, characterized in that the discharging composition is first applied onto the fabric textile and the first composition containing - the dischargeable dye is deposited upon said discharging composition.

7. A process as claimed in any one of the preceding claims, characterized in that after having applied the first and the discharge composition, the fabric is subjected to heat treatment at a temperature exceeding 80°C and less than the decomposing temperature of the textile material, preferably to a steam treatment at a temperature of 150 to 180°C.

## Patentansprüche

1. Verfahren zum Drucken von polyesterhaltigen Textilmaterialien durch Aufbringen in einer Stufe naß auf naß einer ersten Zusammensetzung, enthaltend wenigstens eine ätzbaren Farbstoff und eine Ätzzusammensetzung, welche eine Verbindung enthält, die den ätzbaren Farbstoff atzt, auf einen Stoff, Trocken des Stoffs und Fixieren der Farbstoffe durch Erwärmen, dadurch gekennzeichnet, daß der ätzbare Farbstoff durch eine Thioharnstoff- oder Isothioharnstoffverbindung, welche in der Ätzzusammensetzung vorliegt, geätzt wird.

2. Verfahren nach Anspruch 1, dadurch gekennzeichnet, daß die Ätzzusammensetzung höchstens 4 % eines farbstoffätzenden Metallsalzes als zusätzliches Ätzmittel neben 0,1-10 % einer Thioharnstoff- oder Isothioharnstoffverbindung als Ätzmittel enthält.

3. Verfahren nach Anspruch 2, dadurch gekennzeichnet, daß das farbstoffätzende Metallsalz ein Halogenid eines Metalls der zweiten bis vierten Gruppe des Periodensystems ist.

4. Verfahren nach Anspruch 2 oder 3, dadurch gekennzeichnet, daß die Ätzzusammensetzung 0,1-5 % einer Thioharnstoff- oder Isothioharnstoffverbindung als Ätzmittel enthält.

5. Verfahren nach einem der Ansprüche 2 bis 4, dadurch gekennzeichnet, daß das Metallhalogenid Zink- oder Zinnchlorid ist.

6. Verfahren nach einem der vorhergehenden Ansprüche, dadurch gekennzeichnet, daß die Ätzzusammensetzung zuerst auf das Gewebe aufgebracht wird und die erste Zusammensetzung, die den ätzbaren Farbstoff enthält, auf der Ätzzusammensetzung abgeschieden wird.

7. Verfahren nach einem der vorhergehenden Ansprüche, dadurch gekennzeichnet, daß nach dem Aufbringen der ersten Zusammensetzung und der Ätzzusammensetzung der Stoff einer Wärmebehandlung bei einer Temperatur oberhalb 80°C und unterhalb der Zersetzungstemperatur des Textilmaterials, vorzugsweise einer Dampfbehandlung bei einer Temperatur von 150 bis 180°C, ausgesetzt wird.

## Revendications

1. Procédé d'impression de matériaux textiles contenant du polyester, qui consiste à appliquer en une étape suivant la technique à l'humide une première composition contenant au moins un colorant sensible à l'attaque d'un rongeant et une composition d'enlevage contenant un composé de rongeage dudit colorant sensibles à l'attaque d'un rongeant, sur un tissu, à sécher le tissu et à fixer les colorants par chauffage, caractérisé en ce que le colorant sensible à l'attaque d'un rongeant est soumis à l'effet d'enlevage d'une thiourée ou d'une isothiourée présente dans la composition d'enlevage.

2. Procédé selon la revendication 1, caractérisé en ce que la composition d'enlevage contient, outre 0,1 à 10 % d'une thiourée ou isothiourée à titre d'agent de rongeage, jusqu'à 4 % d'un sel métallique de rongeage de colorant à titre d'agent de rongeage additionnel.

3. Procédé selon la revendication 2, caractérisé en ce que le sel métallique de rongeage de colorant est un halogénure d'un métal du second au quatrième groupe du Tableau Périodique.

4. Procédé selon la revendication 2 ou 3, caractérisé en ce que la composition d'enlevage contient de 0,1 à 5 % d'une thiourée ou isothiourée à titre d'agent de rongeage.

5. Procédé selon les revendications 2 à 4, caractérisé en ce que l'halogénure métallique est le chlorure de zinc ou le chlorure stanneaux.

6. Procédé selon l'une quelconque des revendications précédentes, caractérisé en ce que la composition d'enlevage est d'abord appliquée sur un tissu textile, la première composition contenant le colorant sensible à l'attaque d'un rongeant étant déposée sur cette composition d'enlevage.

7. Procédé selon l'une quelconque des revendi- . cations précédentes, caractérisé en ce que postérieurement à l'application de la première composition et de la composition d'enlevage, le tissu est soumis à un traitement thermique à une température supérieure à 80°C et inférieure à la température de décomposition du matériau textile, de préférence à un traitement par la vapeur à une température de 150 à 180°C.
